

# UNITED STATES PATENT OFFICE.

CHRISTOPHER ZUG, OF PITTSBURG, PENNSYLVANIA.

## MANUFACTURE OF WROUGHT-IRON.

SPECIFICATION forming part of Letters Patent No. 294,949, dated March 11, 1884.

Application filed June 18, 1883. (No specimens.)

*To all whom it may concern:*

Be it known that I, CHRISTOPHER ZUG, a citizen of the United States, residing at Pittsburgh, county of Allegheny, State of Pennsylvania, have invented or discovered a new and useful Improvement in Manufacture of Wrought-Iron; and I do hereby declare the following to be a full, clear, concise, and exact description thereof.

10 My invention relates to the manufacture of wrought-iron by the use of scrap-steel in connection with the ordinary puddling or boiling operation or process, and is directed to the improvement of the quality of the product, so as to secure in such product a greatly increased tensional or torsional strength without impairment of its welding qualities.

15 In working my improved process I make use of puddling or boiling furnaces, or any furnace suitable for puddling or boiling iron in the known methods of doing such work, and in such furnaces I carry on the ordinary puddling or boiling operation in the way or manner common where the resultant product is to be balled and then removed; but at 20 or about the time, or preferably a little before, the iron under such treatment "comes to nature," as it is called, or has reached, by what may be termed a "process of agglutination," such condition that it is ready to be worked up into balls or to form the rudiments of a ball, I then charge into the mass of molten metal any desired quantity of scrap-steel or steel cut into comparatively small pieces, and 25 in the proportion of about from five to twenty-five per cent., by weight, of such steel as compared with the molten iron under treatment. While some variation in percentage may be allowed, according to the quality of product desired, the proportions employed should not 30 differ materially from those above stated. The scrap-steel thus introduced is by the use of a suitable rabble or tool worked up or intermingled with the iron under treatment, so as to become fused and be thoroughly intermingled 35 with it, or the steel being first melted, or taken as it is produced in the crucible or open hearth, may be charged into and, by stirring, be diffused through the material, as above set forth. 40

45 50 In either case the balling proceeds from that point on in the usual way.

I have found as a result of practical working that I am enabled by this process largely to increase the strength of the product manu-

factured as regards its capacity to resist both 55 tensional and torsional strains, and at the same time without destroying or materially impairing the welding properties peculiar to wrought-iron. I am not able to state with certainty 60 the chemical combinations which govern this result, but have merely found it to be a fact. I submit, however, as a matter of theory, that in thus mixing scrap-steel with molten iron, just at or about the time it comes to nature, some of the characteristic features of steel 65 peculiar to the chemical combination therewith of its carbon may be so diffused through and added to the iron as to impart thereto a greater or less percentage of such qualities, but without so changing its condition, state, or chemical 70 composition as to affect materially that distinctive quality of wrought-iron by which it is capable of being welded without a flux; hence the amount of steel to be added should 75 in no case be so great as to give a non-weldable product.

I am aware that it is not new to employ scrap-steel in the manufacture of steel, and I am also aware that it is not new to mix together, melt, and puddle pig-iron and scrap-steel for the production of malleable iron, and 80 I am further aware that it is old to refine iron by the Bessemer or other process, and mix steel therewith when it comes to nature in a puddling-furnace, and that it is also old to mix 85 and melt Bessemer or scrap steel in equal proportions, and to combine this compound with pig-iron in the puddling operations; but I am not aware that it has ever been attempted to improve the quality of wrought-iron by adding scrap-steel thereto, in about the proportions stated, at or near the end of the puddling process, or when it comes to or approaches 90 nature.

I claim herein as my invention— 95  
The process of improving the quality of wrought-iron without destroying its weldable quality as such by intermixing steel therewith, in about the proportions specified, during the puddling or boiling process, as it comes 100 to or approaches nature, substantially as described.

In testimony whereof I have hereunto set my hand.

CHRISTOPHER ZUG.

Witnesses:

R. H. WHITTLESEY,  
C. M. CLARKE.